

## UNITED STATES PATENT OFFICE

2,517,111

LIGHT-SENSITIVE BLUEPRINT LAYER AND  
PROCESS OF PRODUCING THE SAME

Edward Jahoda, Manhasset, N. Y.

No Drawing. Application November 14, 1946,  
Serial No. 709,786

3 Claims. (Cl. 95—7)

**1** This invention relates to a light sensitive layer and to the art of making it. More specifically, it relates to a light sensitive blueprint layer and to a method of making blueprints.

Blueprints are reproductions on paper or other suitable base materials such as cloth, film, metal etc., which are produced by applying to the base, either directly or after a precoat, a layer that contains light-sensitive iron compounds and that is freely soluble in water unless exposed to light. By exposing the layer to actinic light while in contact with a selectively light pervious original, the exposed portions of the layer become more or less insoluble in water depending upon the nature

**2** combination of ferrous salts and ferricyanide compounds; yet this combination is neither light-sensitive nor soluble and therefore not useful for blueprint layers. Typical iron salts used for blueprints are ferric ammonium citrate, ferric ammonium oxalate, ferric sodium oxalate, ferrous oxalate, ferrous ammonium oxalate; typical iron cyanide compounds are potassium ferricyanide, potassium sodium ferricyanide, potassium ferrocyanide.

According to the different starting combinations of iron salts and iron cyanide compounds that form the blue pigment the following types of blueprint layers can be formulated:

| Blueprint layer containing |               |                        |                        | to be designated as | color of layer before exposure |
|----------------------------|---------------|------------------------|------------------------|---------------------|--------------------------------|
| ferrous salts              | ferrous salts | ferricyanide compounds | ferricyanide compounds |                     |                                |
| X                          |               | X                      | X                      | A-type              | yellow.                        |
| X                          |               | X                      | X                      | B-type              | blue.                          |
| X                          |               | X                      | X                      | C-type              | Do.                            |
| X                          | X             | X                      | X                      | AB-type             | green, grey or blue.           |
| X                          | X             | X                      | X                      | AC-type             | green or blue.                 |
| X                          | X             | X                      | X                      | BC-type             | blue.                          |

and intensity of the light and upon the duration of the exposure. After the exposure the unexposed, and therefore, still soluble portions of the layer are removed by washing whereby the base is laid bare in the state and color it possessed before the light-sensitive layer was applied. Finally, the insoluble portions of the layer which have not been removed by the washing operation are transformed into pigmented areas of a blue color by oxidation in the air or in a developing solution. As the markings of the original correspond to the washed-out portions of the layer, positive originals yield prints with white lines and a blue background—blueprints in the narrow sense, and negative originals yield prints with blue lines and a white background—blueline prints. In the following the term blueprint is used in the wider sense including blueline prints.

The blue pigment of the finished prints consists mostly of Prussian blue of the general composition  $\text{Fe}^{''''}[\text{Fe}^{''''}\text{Fe}^{''''}(\text{CN})_6]_3$ . It can be formed from each one of the following combinations of iron salts and iron cyanide compounds which differ in regard to the initial valency state of the components:

- (A) Ferric salts and ferricyanide compounds,
- (B) Ferric salts and ferrocyanide compounds,
- (C) Ferrous salts and ferricyanide compounds.

Prussian blue can also be formed from a com-

30 The A, B and C types are "pure layers," the AB, AC and BC type may be called mixed layers. At the inception of the art only the A-type layers were known; they were used exclusively during the major part of that period and they are still in wide use at the present. About a decade ago the AB-type layers and more recently the "pure" B-type layers were introduced to meet the demands for a "latitude" paper, that is a blueprint paper by which good prints could be obtained at the same printing speed, from ink and pencil drawings, from old and new tracings and from originals of different transparency. The "pure" and "mixed" C-type layers are the latest types; 40 they excel the A-type layers in brilliancy and depth of color and the AB- and B-type layers in latitude. However as yet they have not been used to any great extent since they cannot be stored for a greater length of time and are not capable of a perfect wash-out.

Iron salts and iron cyanide compounds are the sole indispensable components in the formation of the blue pigment. Yet other ingredients which do not enter into the formation of the pigment proper, such as buffers, oxidizers, thickeners, wetting agents, etc., are employed for various purposes, for instance, in order to stabilize the pH of the sensitizing solution, to reduce its penetration or to modify its wetting characteristics, also in order to control contrast or speed, to im-

## 3

prove the keeping qualities of the layer before the exposure, and to insure a proper wash-out of the soluble portions.

For all practical purposes good keeping qualities and a proper wash-out are just as important requirements of blueprint layers as a pleasing dark blue color obtained at satisfactory printing speeds.

Slow printing layers, especially of the A-type, usually have good keeping and wash-out qualities without requiring substantial amounts of non-pigment forming substances; they contain a relatively large amount of free ferricyanide which, of itself, slows down the printing speed, contributes to the formation of the pigment, insures good keeping qualities, and facilitates the wash-out. Fast printing layers, however, especially those which are not of the A-type, contain little or no free ferricyanide. They require substantial amounts of non-pigment forming substances to improve the keeping and the wash-out qualities of the layers. For this purpose numerous substances have been employed, such as neutral alkali oxalates, alkaline hydrolyzable alkali metal compounds, acid hydrolyzable alkali metal phosphates, persulfate compounds, sugars and oxidizing agents. These substances, in the first place, have the drawback that they tend to impair the brilliancy and the depth of the blue and to reduce the printing speed. Further, though of limited use on A, AB and B-type layers, these substances do not give satisfactory results on "pure" and "mixed" C-type layers or do so only if employed in such large amounts as to offset the distinct advantages of the C-type layers.

It is the object of this invention to improve the keeping and wash-out qualities of blueprint layers without impairing color or printing speed.

Another more specific object of the invention is the improvement of the keeping and wash-out qualities of the "pure" and "mixed" C-type blueprint layers up to and above the standards set by the other types of blueprint layers without impairment of their advantages, particularly in respect to brilliancy of color, depth of color and latitude.

In other words, it is an object of this invention to overcome obstacles now in the way of a broad use of "pure" or "mixed" C-type blueprint layers.

A further object of the invention is an improved "latitude" blueprint paper with good keeping and wash-out qualities.

I have found that the neutral alkali metal hexametaphosphates impart excellent keeping and wash-out qualities to all types of blueprint layers including the "pure" and "mixed" C-type layers. They can be used effectively in greatly varying amounts depending upon the type of layer. Certain B-type layers do not require more than 5% of hexametaphosphates by weight of the total solids, certain BC-type layers require as much as 20%. Up to 20%, these compounds do not affect measurably the printing speed. Up to 50% they do affect the speed but do not affect visibly the brilliancy and the depth of the blue; therefore they can be utilized to control the printing speed of blueprint layers.

Neutral alkali metal hexametaphosphates are commercially available as sodium hexametaphosphate  $\text{Na}_2\text{Na}_4(\text{PO}_3)_6$ , which is sold under the trademark "Calgon" (unadjusted grade), and as a potassium sodium hexametaphosphate of the composition  $\text{K}_2\text{Na}_4(\text{PO}_3)_6$  or  $\text{KNa}_5(\text{PO}_3)_6$ , sold under the trademark "Plastic Metaphosphate."

Whereas "Calgon" can be used just as well as

the "Plastic Metaphosphate" in so far as the improvement of keeping and wash-out qualities is concerned, I prefer in most cases to use the "Plastic Metaphosphate" because this potassium sodium hexametaphosphate forms an aqueous solution of high viscosity. It offers a convenient way to increase the viscosity of the blueprint solution which is desirable for most commercial grades of base papers. A solution of higher viscosity acts the same way as a harder sizing of the base sheet, that is, it reduces the rate of penetration into the base; it is well known that thus the appearance of the blue color is improved. The use of "Plastic Metaphosphate," therefore, dispenses with the need for other thickeners.

Tentatively, the beneficial effects of the alkali metal hexametaphosphates on the keeping and wash-out qualities of blueprint layers may be attributed to the formation of complex molecules by the same mechanism that causes their effective peptizing and dispersing action upon many solid materials, including heavy metal salts and oxides. It may be assumed that the complex compounds formed are fairly weak and that they are destroyed by the exposure to light, which also would account for the fact that even large amounts of the alkali metal hexametaphosphates will not impair the brilliancy and depth of the blue pigment.

The following examples are given to illustrate my invention:

*Example 1.—(B-type layer of very fast printing speed)*

25 5.5 grams of "Plastic Metaphosphate" are dissolved at room temperature under vigorous stirring in 120 cc. of water. To this solution are added and dissolved in conventional manner 4.5 grams of potassium oxalate, 20 grams of iron ammonium oxalate and 5 grams of potassium ferrocyanide.

40 The resulting layer keeps very well even under unfavorable storing conditions, the wash-out is excellent. Without "Plastic Metaphosphate" the washed-out portions of the layer show a considerable blue stain. "Calgon" may be substituted for the "Plastic Metaphosphate."

*Example 2.—(C-type layer of slow printing speed)*

55 5.5 grams of "Plastic Metaphosphate" are dissolved at room temperature under vigorous stirring in 80 cc. of water. Next there are added 3.8 grams of potassium sodium ferricyanide and then 4 grams of ferrous ammonium oxalate. The stirring action must be continued until the solution turns dark blue. This solution must be filtered but need not be heated.

60 The resulting layer has good keeping and wash-out qualities. Without the "Plastic Metaphosphate" the wash-out is very poor and the layer spoils completely within a very few days even under ideal storing conditions. In this example the "Plastic Metaphosphate" acts also as speed reducing agent. "Calgon" may be substituted for the "Plastic Metaphosphate."

*Example 3.—(BC-type layer of fast printing speed)*

70 A solution prepared as in Example 1, and a solution according to Example 2, are mixed.

The resulting layer has an extremely great latitude. The keeping and wash-out qualities are better than those of conventional layers of much slower printing speeds.

The alkali metal hexametaphosphates used according to my invention are neither alkaline nor acid hydrolyzable salts. They are practically neutral and stable in solution. They can be used in excessive amounts without impairing the blue pigment or staining the washed-out portions.

Alkaline hydrolyzable salts are able to improve the keeping and wash-out qualities of blueprint layers. Yet if used in more than in definite small amounts they affect the blue pigment under formation of brownish decomposition products of basic iron. They tend to dull the blue color and to stain the washed-out portions brownish.

Acid hydrolyzable salts are able to improve the wash-out qualities of blueprint layers. Yet they are unable to improve the keeping qualities; if used in more than in definite small amounts they affect the keeping qualities adversely. They tend to stain the washed-out portions bluish.

With the neutral alkali metal hexametaphosphates a hitherto unknown flexibility in the formulation of blueprint layers can be achieved.

What I claim is:

1. A sensitized solution having relatively high viscosity for a blueprint paper coating with a relatively reduced rate of penetration into the base paper containing approximately 5 parts of neutral hydrolyzable potassium sodium hexametaphosphate, approximately 4 parts of alkali ferricyanide, and approximately 4 parts of a weak dissociable ferrous salt in solution.

2. A sensitized solution having relatively high viscosity for a blueprint paper coating with a relatively reduced rate of penetration into the

35

base paper containing approximately 5½ parts of neutral hydrolyzable potassium sodium hexametaphosphate, approximately 3½ to 4 parts of potassium sodium ferricyanide, and 4 parts of ferrous ammonium oxalate in solution.

3. The process of producing a coating for blueprint paper having a viscosity high enough to reduce the rate of penetration into the base paper comprising dissolving approximately 5½ parts of neutral hydrolyzable potassium sodium hexametaphosphate into approximately 80 parts of water, adding approximately 3.8 parts of potassium ferricyanide, adding approximately 4 parts of ferrous ammonium oxalate at room temperature, agitating the resultant solution until the solution reacts to produce a dark blue color, and applying the resultant solution to a paper base whereby a layer having good keeping and wash-out qualities is provided the blueprint paper.

20

EDWARD JAHODA.

#### REFERENCES CITED

The following references are of record in the file of this patent:

25

#### UNITED STATES PATENTS

| Number       | Name     | Date           |
|--------------|----------|----------------|
| 2,093,738    | Reynolds | Sept. 21, 1937 |
| 2,126,504    | Reynolds | Aug. 9, 1938   |
| 30 2,172,216 | Miller   | Sept. 5, 1939  |

30

#### FOREIGN PATENTS

| Number  | Country       | Date          |
|---------|---------------|---------------|
| 461,893 | Great Britain | Feb. 22, 1937 |

35